

## UNITED STATES PATENT OFFICE

1,999,212

## LUBRICATING OIL

John E. Schulze, Chicago, Ill., assignor to Red River Refining Company, Inc., Chicago, Ill., a corporation of Louisiana

No Drawing. Application August 24, 1931,  
Serial No. 559,120

19 Claims. (Cl. 196—151)

This invention relates to lubricating oils; and it relates more particularly to novel lubricating oils, especially those produced from paraffin base crudes, which are obtainable by the process disclosed and claimed in this applicant's prior application, Serial No. 544,931, filed March 18, 1922 (now Patent No. 1,448,709, March 13, 1923), and which are also disclosed in applicant's prior co-pending application Serial No. 624,826, filed March 13, 1923, of both of which prior applications the present application is a continuation in part. In said prior Patent No. 1,448,709 there was disclosed a novel process of distilling petroleum, distillates and residua under very low absolute pressure and under non-oxidizing conditions, the distillation pressure most desirably being maintained as low as 2 to 4 millimeters mercury absolute and not exceeding 25 millimeters mercury absolute as a practical maximum. Said process enables the production of novel distillates, particularly lubricating oil distillates, that are characterized by narrow viscosity range and boiling point or distillation range, as well as by other desirable properties such as excellent color, and freedom from tarry and asphaltic constituents. The process by which these novel products can be obtained, as well as apparatus suitable for carrying out the process, were fully disclosed in said prior application. Said process and novel products were also claimed therein both broadly and specifically, the specific claims being, however, directed more especially to the novel products derived from naphthene base petroleum. Said prior application also disclosed novel products derived from paraffin base petroleum, but by official requirement it was required that claims to the paraffin base products be divided out. Said application Serial No. 624,826 was therefore filed and directed more particularly to such paraffin base products. As stated in said prior application Serial No. 544,931, the novel process described therein is also applicable to the treatment of topped or stripped crudes and still bottoms of paraffin base origin; but in order to treat such starting materials commercially it is necessary to make special provision for the removal of the paraffin wax content which comes over during the entire distillation. One method of removing paraffin from the distillates is by centrifuging, although it is to be understood that other methods can be employed for this purpose.

In handling paraffin base crudes according to refinery practice prevailing prior to the present invention, it has been customary to distil overhead with steam up to a critical temperature at which decomposition takes place. The distillates thus obtained are freed from their paraffin content, reduced, acid treated, and filtered, to produce commercial products commonly known to the trade as "100 Pennsylvania Neutral", "200 Pennsylvania Neutral", etc. according to the particular viscosity of the commercial grade in question; the highest viscosity known to the trade in this series being 220 seconds at 100° F. The still bottoms (cylinder stock) remaining are freed from amorphous waxy content and filtered to desired color known as "FFP". In contrast to this prior practice, the novel process of the prior application Serial No. 544,931 makes it possible to treat the still bottoms or cylinder stock from paraffin base crudes by distilling overhead without decomposition, and obtaining at least 60% or more of the material in the form of straight overhead lubricating oil distillates ranging in viscosity from 250 up to over 1200 seconds viscosity, Saybolt Universal (at 100° F.), and even as high as 180 seconds Saybolt at 210° F. Moreover, the color of these overhead distillates is far superior to prior commercial lubricating oils of comparable viscosity, the color of the new products of viscosity as high as 1200 seconds (at 100° F.) ranging from 2 to 5 N. P. A. just as the distillates come over and without any further refining treatment. These novel products are also of exceptionally high flash and fire test and are free of tarry matter, giving no precipitate with the standard precipitation test. This test, as is well known, consists in shaking a measured quantity of the oil with a measured quantity of a known solvent such as gasoline and allowing the mixture to stand for a definite length of time. Furthermore the novel products show an exceptionally low carbon residue by the Conradson carbon test.

The residuum or still bottoms remaining after distillation of the novel lubricating oils in accordance with the novel process is an extremely heavy cylinder stock of a viscosity that may be as high as 250 seconds Saybolt (at 210° F.) with a flash point of 630° F. and 700° F. fire test never having been obtained heretofore except by cracking and wasting lubricating fractions which are now obtainable by the process of said Patent 1,448,709 as finished overhead lubricating oil distillates.

For the sake of illustration examples of certain new paraffin base lubricating oils that are typical of those comprised in the invention will now be given, but it is to be understood that the invention is not limited to these specific oils. Data will be given first for two typical light motor oils corresponding to established commercial grades known as 150 viscosity and 200 viscosity, and comparative data will be given for the best obtainable corresponding oils of the prior art. It is to be understood that a variation of about 5 seconds plus or minus from a commercial viscosity grade is customarily permissible so that in

referring to a 150 viscosity oil, for example, this is to be taken as approximate and as including a range of 145 to 155 viscosity in practice.

| 5  | Paraffin base                                  |                      | 10            |
|----|------------------------------------------------|----------------------|---------------|
|    | New oils                                       | Prior oils<br>(best) |               |
| 10 | 150 viscosity type                             |                      |               |
|    | Gravity (Baumé)                                | 31.0                 | 31.5          |
|    | Viscosity range (at 100° F.)                   | 100 sec.             | Over 540 sec. |
|    | Distillation range<br>(At 2 to 5 mm. absolute) | 50° F.               | Over 130° F.  |
|    | Conradson carbon                               | 0.015%               | 0.04%         |
| 15 | Color (N. P. A.)                               | 1                    | 2             |
|    | Flash point                                    | 410° F.              | 400° F.       |
|    | Fire point                                     | 470° F.              | 450° F.       |
|    | Cold test                                      | 25° F.               | 25° F.        |
| 20 | 200 viscosity type                             |                      |               |
|    | Gravity                                        | 29.7                 | 31.1          |
|    | Viscosity range (at 100° F.)                   | 100 sec.             | Over 600 sec. |
|    | Distillation range<br>(At 2 to 5 mm. absolute) | 60° F.               | Over 140° F.  |
|    | Conradson carbon                               | 0.03%                | 0.07%         |
|    | Color (N. P. A.)                               | 1.5                  | 2.0           |
|    | Flash point                                    | 430° F.              | 420° F.       |
|    | Fire point                                     | 500° F.              | 475° F.       |
|    | Cold test                                      | 25° F.               | 20° F.        |

| 25 | Baumé gravity | Viscosity (at 10° F.) | Flash point ° F. | Fire point ° F. | Cold test ° F. | Color N. P. A. | Conradson carbon residue percent | 25 |
|----|---------------|-----------------------|------------------|-----------------|----------------|----------------|----------------------------------|----|
| 30 | 30.0          | 250                   | 450              | 510             | 25             | 2.0            | 0.05                             | 30 |
|    | 29.5          | 300                   | 465              | 525             | 25             | 2.0            | 0.06                             |    |
|    | 29.0          | 400                   | 420              | 540             | 25             | 2.5            | 0.08                             |    |
|    | 28.8          | 600                   | 500              | 580             | 25             | 2.5            | 0.10                             |    |
|    | 28.6          | 800                   | 610              | 570             | 25             | 2.5            | 0.15                             |    |
|    | 28.4          | 1000                  | 520              | 580             | 25             | 3.0            | 0.20                             |    |
| 35 | 28.0          | 1200                  | 640              | 600             | 25             | 3.0            | 0.25                             | 35 |

By the term "viscosity range", as herein employed is to be understood the difference in viscosity between the first 10% fraction and the last 10% fraction obtained by distilling a sample of the oil at or below 5 (e. g. at from 2 to 5) millimeters mercury absolute pressure and under non-oxidizing conditions. While this viscosity range is always much narrower for the new oils than for the oils of the prior art, it is not to be inferred that it must necessarily be as narrow in all cases as in the specific examples given above. For example, in the case of a novel 150 viscosity oil, the viscosity range may even be as great as 420 seconds while still being sharply differentiated from the prior art oils of this commercial grade, while on the other hand a viscosity range as low as 65 seconds is obtainable. Similarly a viscosity range of as much as 500 seconds for a novel oil of the 200 viscosity type is still within the scope of the invention although ordinarily such oil is characterized by a much narrower viscosity range, say, 50 to 100 seconds. In the same way, the distillation ranges of 50° to 60° F. above specified for the novel 150 and 200 viscosity oils are not to be understood as limiting, a range of from 15° to 75° F. in oils of these types being permissible within the scope of the invention; but ranges of from 25° to 75° F., and especially of from 25° to 60° F., are more particularly representative. Likewise the carbon residue by the Conradson test may in some cases be as much as 0.02% for the 150 viscosity oil and as high as 0.04% for the 200 viscosity oil, even these maximum percentages being obviously far below those for the corresponding grades of prior art oils. More usually

the novel lubricating oils having a viscosity of 150 seconds (at 100° F.) or less leave a Conradson carbon residue of from 0.005 to 0.015 per cent; while those whose viscosity approaches 200 seconds leave a carbon residue of from 0.01 to 0.03 per cent.

It may be noted that the novel oils of the viscosities given in the above tables are ideal starting material for the manufacture of white medicinal oils, and that the medicinal oils resulting from the use of these starting materials are in themselves novel and readily distinguishable by their physical constants from white medicinal oils heretofore known. These new medicinal oils are not however specifically claimed in the present application.

As illustrating the character of typical novel paraffin base oils of higher viscosities (i. e. above 220 seconds Saybolt at 100° F.) that are also comprised within the present invention, data of a series of such oils (medium, heavy and extra heavy) of different typical viscosities is given below:

The typical oils of which the physical constants are shown in this last table are strictly straight run overhead distillates, a fact that cannot be too strongly emphasized, since it radically and fundamentally distinguishes them from prior art oils of corresponding viscosities, all of which have heretofore been manufactured by blending with a heavy cylinder stock or still bottoms enough of a lighter overhead lubricating distillate to obtain the viscosity called for by commercial specifications. Accordingly such prior art commercial oils having viscosities exceeding 220 seconds (at 100° F.) have in every instance been characterized by exceedingly wide viscosity and distillation ranges, which have been inherently essential characteristics of these oils. The color of these prior art oils has also been relatively poor because of the necessity for including the heavy cylinder stock in blending, this cylinder stock being usually of a very dark color. Furthermore the Conradson carbon test of these blended oils is always relatively high, the figure necessarily depending upon the percentage of the cylinder stock employed in the blend. In such blended oils the Conradson carbon customarily runs from a minimum of about 0.20% for a 250 viscosity oil to a maximum of well over 1% for heavier viscosities. In contrast to this, oils of the present invention whose viscosities are from 220 seconds up to 400 seconds, or even as high as 800 seconds (at 100° F.), leave a carbon residue by the Conradson carbon test usually not exceeding 0.15 per cent, and in some cases not exceeding 0.01 per cent. Those whose viscosities lie between 400 and 600 seconds commonly leave a Conradson carbon residue of from 0.015 to 0.15 per cent. For those having viscosities between

600 and 900 seconds the residue usually is from 0.05 to 0.25 per cent. Among the still heavier oils of the present invention, whose viscosity is customarily measured at 210° F., those of viscosity 5 between 75 and 100 seconds at 210° F. leave a carbon residue of from 0.2 to 0.6 per cent; of viscosity between 100 and 130 seconds, a residue of from 0.5 to 0.9 per cent; and of viscosity between 130 and 180 seconds, a residue of from 0.8 to 1.2 per cent. In every case, these figures are far below those for previously known oils of corresponding viscosity. It may be noted here that a viscosity of 900 seconds Saybolt Universal at 100° F. is equivalent to 75 seconds Saybolt Universal 15 at 210° F.

The table above given shows that other physical constants of the aforesaid new oils of viscosities higher than 220 seconds (at 100° F.) also sharply distinguish them from the blended oils of the 20 prior art. It is not to be understood that the new oils are limited to the particular viscosity specified since these are only typical cuts obtainable by the new process. Taking the specific 25 cuts given in the table, the viscosity range (i. e. the difference in viscosity between the first and last 10 per cent fractions obtained by distilling a sample) for any one of these oils does not ordinarily exceed 150 seconds Saybolt Universal (at 100° F.), and for the viscosities above 400 30 still lower viscosity ranges are the rule, a viscosity range as small as 100 seconds for the highest viscosity (1200) given in the table being characteristic. A viscosity range of about 50 seconds (at 100° F.) is practically the minimum for oils 35 of these types, and a viscosity range of between 50 and 250 seconds (at 100° F.) characterizes most of them. It is of course permissible within the invention to combine a number of the above 40 cuts given in the table into a single cut, or into two or more. Even if all the distillates given in 45 the last table were to be combined into a single cut, the viscosity range of this cut would in practice be not more than about 1200 seconds which is very much less than the lowest viscosity range possible in the best oils of comparable viscosities heretofore known in the art.

It is to be noted also that, like the lighter oils given in the first table, all the new heavier hereinabove mentioned oils also distill over substantially completely (i. e. 98%) without substantial cracking at or below 5 (e. g. 2 to 5) millimeters mercury absolute pressure and under non-oxidizing conditions, without exceeding about 650° F. as a maximum distilling temperature or 50 end point, the minimum end point for novel oils of this type under such conditions being about 450° F. When the prior art blended oils are subjected to distillation under these conditions, on the other hand, they do not distil over substantially completely, but on the contrary a very substantial percentage remains as a residuum, the amount of this residuum depending upon the amount of heavy cylinder stock employed in the blend. Expressed generally, the amount of 55 a prior art blended oil that will distil over under these conditions can be expressed by the formula  $A + 80\%$  (approximately) of  $B$ , where  $A$  is the proportion of light overhead and  $B$  is the proportion of heavy cylinder stock used in the blend. This is evidently another convenient way of sharply distinguishing the new oils from the old.

Reference herein to an oil as having a given viscosity signifies the viscosity of a test sample 60 determined in the usual way by means of a

standard viscosimeter. This figure is in fact the mean or average viscosity of the oil in question. This should be distinguished from the "viscosity range" of the same oil which is hereinabove defined and is used also in certain of the appended 5 claims to aid in defining the novel oils of the invention.

What I claim is:

1. As a new article of manufacture, a straight overhead paraffin base lubricating oil distillate 10 having a viscosity of not less than approximately 150 seconds Saybolt Universal (at 100° F.), said distillate being a high-grade finished lubricating oil product obtained directly by high vacuum distillation at absolute pressure not exceeding 25 15 millimeters of mercury, without acid treatment or filtration, and being further characterized by the fact that a sample thereof distils substantially completely at from 2 to 5 millimeters mercury absolute pressure and under non-oxidizing 20 conditions between temperatures differing only by from about 25° to 75° F.

2. As a new article of manufacture, a straight overhead paraffin base lubricating oil distillate 25 having a viscosity of not less than 150 seconds Saybolt Universal (at 100° F.), said distillate being a high-grade finished lubricating oil product obtained directly by high vacuum distillation at absolute pressure not exceeding 25 millimeters 30 of mercury, without acid treatment or filtration, and being further characterized by the fact that when a sample of said oil is substantially completely distilled under an absolute pressure of from 2 to 5 millimeters of mercury and under non-oxidizing 35 conditions, the first ten per cent fraction and the last ten per cent fraction of the distillate differ in viscosity only by from about 50 to 250 seconds Saybolt Universal (at 100° F.).

3. As a new article of manufacture, a straight overhead paraffin base lubricating oil distillate 40 having a viscosity of at least about 200 seconds Saybolt Universal (at 100° F.), said distillate being a high-grade finished lubricating oil product obtained directly by high vacuum distillation at absolute pressure not exceeding 25 millimeters 45 of mercury, without acid treatment or filtration, and leaving a carbon residue by the Conradson carbon test of from 0.01 to about 0.04 per cent.

4. As a new article of manufacture, a straight overhead paraffin base lubricating oil distillate 50 having a viscosity approximating 200 seconds Saybolt Universal (at 100° F.), said distillate leaving a carbon residue by the Conradson carbon test of from 0.01 to 0.03 per cent, said distillate being a high-grade finished lubricating oil product obtained directly by high vacuum distillation at 55 absolute pressure not exceeding 25 millimeters of mercury, without acid treatment or filtration, and being further characterized by the fact that a sample thereof distils substantially completely at from 2 to 5 millimeters mercury absolute pressure and under non-oxidizing conditions between 60 temperatures differing by from 25° to about 60° F., the first ten per cent fraction and the last ten per cent fraction of the sample differing in viscosity by from 50 to about 100 seconds Saybolt 65 Universal (at 100° F.).

5. As a new article of manufacture, a straight overhead paraffin base lubricating oil distillate having a viscosity higher than 220 seconds Saybolt Universal (at 100° F.), said distillate being a high-grade finished lubricating oil product obtained directly by high vacuum distillation at absolute pressure not exceeding 25 millimeters of mercury, without acid treatment or filtration, and 70

being further characterized by the fact that a sample thereof distils substantially completely at from 2 to 5 millimeters mercury absolute pressure under non-oxidizing conditions with a maximum distilling temperature or end point of from 450° to 650° F.

6. As a new article of manufacture, a straight overhead paraffin base lubricating oil distillate having a viscosity lying between 220 and 400 seconds Saybolt Universal (at 100° F.), said distillate being a high-grade finished lubricating oil product obtained directly by high vacuum distillation at absolute pressure not substantially exceeding 25 millimeters of mercury, without acid treatment or filtration, and leaving a carbon residue of from about 0.01 to 0.15 per cent by the Conradson carbon test.

7. As a new article of manufacture, a straight overhead paraffin base lubricating oil distillate having a viscosity lying between 400 and 600 seconds Saybolt Universal (at 100° F.), said distillate being a high-grade finished lubricating oil product obtained directly by high vacuum distillation at absolute pressure not substantially exceeding 25 millimeters of mercury, without acid treatment or filtration, and leaving a carbon residue of from about 0.015 to 0.15 per cent by the Conradson carbon test.

8. As a new article of manufacture, a straight overhead paraffin base lubricating oil distillate having a viscosity lying between 600 and 900 seconds Saybolt Universal (at 100° F.), said distillate being a high-grade finished lubricating oil product obtained directly by high vacuum distillation at absolute pressure not substantially exceeding 25 millimeters of mercury, without acid treatment or filtration, and leaving a carbon residue of from about 0.05 to 0.25 per cent by the Conradson carbon test.

9. As a new article of manufacture, a straight overhead paraffin base lubricating oil distillate having a viscosity lying between 75 and 100 seconds Saybolt Universal (at 210° F.), said distillate being a high-grade finished lubricating oil product obtained directly by high vacuum distillation at absolute pressure not substantially exceeding 25 millimeters of mercury, without acid treatment or filtration, and leaving a carbon residue of from 0.2 to 0.6 per cent by the Conradson carbon test.

10. As a new article of manufacture, a straight overhead paraffin base lubricating oil distillate having a viscosity lying between 100 and 130 seconds Saybolt Universal (at 210° F.), said distillate being a high-grade finished lubricating oil product obtained directly by high vacuum distillation at absolute pressure not substantially exceeding 25 millimeters of mercury, without acid treatment or filtration, and leaving a carbon residue of from 0.5 to 0.9 per cent by the Conradson carbon test.

11. As a new article of manufacture, a straight overhead paraffin base lubricating oil distillate having a viscosity lying between 130 and 180 seconds Saybolt Universal (at 210° F.), said distillate being a high-grade finished lubricating oil product obtained directly by high vacuum distillation at absolute pressure not substantially exceeding 25 millimeters of mercury, without acid treatment or filtration, and leaving a carbon residue of from 0.8 to 1.2 per cent by the Conradson carbon test.

12. As a new article of manufacture, a straight overhead paraffin base lubricating oil distillate having a viscosity exceeding 220 seconds Say-

bolt Universal (at 100° F.), said distillate being a high-grade finished lubricating oil product obtained directly by high vacuum distillation without acid treatment or filtration, and being further characterized by the fact that when a sample of said oil is distilled under an absolute pressure of from 2 to 5 millimeters of mercury and under non-oxidizing conditions, the first ten per cent fraction and the last ten per cent fraction differ in viscosity by from about 50 to 1200 seconds Saybolt Universal (at 100° F.).

13. As a new article of manufacture, a straight overhead paraffin base lubricating oil distillate having a viscosity of at least about 220 seconds Saybolt Universal (at 100° F.), said distillate being a high-grade finished lubricating oil product obtained directly by high vacuum distillation without acid treatment or filtration, and being further characterized by the fact that when a sample of said oil is distilled under an absolute pressure of from 2 to 5 millimeters of mercury and under non-oxidizing conditions, the first ten per cent fraction and the last ten per cent fraction differ in viscosity by from about 50 to 150 seconds Saybolt Universal (at 100° F.).

14. As a new article of manufacture, a straight overhead paraffin base lubricating oil distillate having a viscosity of not less than approximately 150 seconds Saybolt Universal (at 100° F.), said distillate being a high-grade finished lubricating oil product obtained directly by high vacuum distillation at absolute pressure not exceeding 25 millimeters of mercury, without acid treatment or filtration, and being further characterized by the fact that a sample thereof distills substantially completely at from 2 to 5 millimeters mercury absolute pressure and under non-oxidizing conditions between temperatures differing only by from 50° to 75° F.

15. As a new article of manufacture, a straight overhead paraffin base lubricating oil distillate as defined in claim 2, the first and last ten per cent fractions of the distilled sample differing in viscosity only by about 100 seconds Saybolt Universal (at 100° F.).

16. As a new article of manufacture, a straight overhead paraffin base lubricating oil distillate having a viscosity of at least about 150 seconds Saybolt Universal (at 100° F.), said distillate being a high-grade finished lubricating oil product obtained directly by high vacuum distillation at absolute pressure not exceeding 25 millimeters of mercury, without acid treatment or filtration, and leaving a carbon residue by the Conradson carbon test of from about 0.015 to 0.02 per cent.

17. As a new article of manufacture, a straight overhead paraffin base lubricating oil distillate as defined in claim 16, leaving a Conradson carbon residue of about 0.015 per cent.

18. As a new article of manufacture, a straight overhead paraffin base lubricating oil distillate having a viscosity of at least about 200 seconds Saybolt Universal (at 100° F.), said distillate being a high-grade finished lubricating oil product obtained directly by high vacuum distillation at absolute pressure not exceeding 25 millimeters of mercury, without acid treatment or filtration, and leaving a carbon residue by the Conradson carbon test of from about 0.03 to 0.04 per cent.

19. As a new article of manufacture, a straight overhead paraffin base lubricating oil distillate having a viscosity approximating 200 seconds Saybolt Universal (at 100° F.), said distillate

leaving a carbon residue by the Conradson carbon test of from about 0.03 to 0.04 per cent, said distillate being a high-grade finished lubricating oil product obtained directly by high vacuum distillation at absolute pressure not exceeding 25 millimeters of mercury, without acid treatment or filtration, and being further characterized by the fact that a sample thereof distils substantially completely at from 2 to 5 millimeters ab-

solute pressure and under non-oxidizing conditions between temperatures differing by from about 60° to about 75° F., the first ten per cent fraction and the last ten per cent fraction of the sample differing in viscosity by from about 100 seconds to 500 seconds Saybolt Universal (at 100° F.).

JOHN E. SCHULZE.